

# UNITED STATES PATENT OFFICE.

JOHN I. CRABTREE, OF ROCHESTER, NEW YORK, ASSIGNOR TO EASTMAN KODAK COMPANY, OF ROCHESTER, NEW YORK, A CORPORATION OF NEW YORK.

## COLORED IMAGE AND PROCESS OF PRODUCING THE SAME

1,389,742.

Specification of Letters Patent. Patented Sept. 6, 1921.

No Drawing.

Application filed May 2, 1919. Serial No. 294,343.

To all whom it may concern:

Be it known that I, JOHN I. CRABTREE, a subject of the King of Great Britain, residing at Rochester, in the county of Monroe 5 and State of New York, have invented certain new and useful Improvements in Colored Images and Processes of Producing the Same, of which the following is a full, clear, and exact specification.

10 My invention relates to colored photographic images and the production thereof. More particularly it relates to the mordanting of dyes onto inorganic compounds which may be dispersed or distributed through a 15 suitable transparent medium in the form of images. For example, I may add to or modify the image of a photographic picture so that a dye will be adsorbed thereon in correspondence with the original image, thus 20 giving a colored image having approximately the same form and gradation as the original picture. The inorganic part of such colored picture may be further treated or removed. Flat or even tones may be similarly 25 changed into colored tints suitable for light filters or general light-modifying purposes. A flat or even tone in the picture being but the image of an object having a flat or even tone. I shall use the word "image" 30 generically to include flat tones as well as the more usual graded images.

The objects of my invention are to effect these results, carry out such a process, and obtain such a product by steps that will be 35 under good control, that will be rapid, that will yield pictures having good gradation, that will not injure or impair the wearing qualities of the product, that will produce stable, clear and brilliant colors, and that 40 will admit of ready duplication of effects, that can be carried on entirely at normal temperatures, that is, in the neighborhood of 70° F., and that can readily be performed by any workman accustomed to ordinary photographic methods. Other objects will hereinafter appear.

Since images made up of silver particles suspended in gelatin are most commonly met with in photographic practice, I will 50 describe, as an example of my invention, its application to a silver image. Generally

stated, I treat the original, a primary image, in such a bath or baths that it is converted into an iron salt, which is capable of mordanting dyes, especially acid dyes of the 55 alizarin series. The methods which will be hereinafter particularly described comprise three principal steps, beginning with the silver photographic image. The silver is first converted into a complex cyanid of silver and iron. In my preferred process this salt is silver ferricyanid, but by the use of other baths silver ferrocyanid may be obtained. This image is then converted into one of a complex cyanid of iron and this 60 in turn into iron hydroxid. This last is a transparent colloidal image and is capable of adsorbing or mordanting dyes, and I specifically enumerate certain acid dyes that may be advantageously used. 65

I will first describe fully the details of my preferred process. A gelatin film in which a silver photographic image is present is bleached in the following bath at 70° F., for about two minutes, whereby the silver 70 is converted into one of silver ferricyanid:

|                        |          |
|------------------------|----------|
| Potassium ferricyanid  | 2 grams. |
| Potassium permanganate | 2 grams. |
| Water to               | 100 cc.  |

Instead of the above bleaching bath the following may be employed:

|                             |         |
|-----------------------------|---------|
| Potassium ferricyanid (10%) | 5 vols. |
| Chromic acid (10%)          | 2 vols. |

85 After being bleached in the above bath the film is washed for about a minute in water and then immersed in the following solution which converts the silver ferricyanid image into a blue image of a complex 90 cyanid of iron together with silver chlorid:

|                   |          |
|-------------------|----------|
| Ferrous sulfate   | 5 grams. |
| Hydrochloric acid | 5 cc.    |
| Water to          | 100 cc.  |

95 The above mentioned bath also has the effect that it dissolves a little manganese stain (manganese dioxid) which was produced by the first named bleaching bath. After rinsing in water, the film is now immersed in a 35% solution of sodium thiosulfate for about a minute, so as to remove the 100

silver chlorid produced in the last bath. It is again rinsed and then immersed in a 1% solution of sodium carbonate or of sodium or potassium hydroxid. The action of this last named bath is to convert the blue image to a faint yellow image of iron hydroxid.

The film containing this image is now placed in the dye solution, and I have found that many dyes, particularly acid dyes of the alizarin series, will be mordanted to the image. The dye bath is composed of a .2% solution of the dye to which acetic acid or ammonia may be added. The following dyes are noted as giving typically good results.

- 15 Alizarin red S
- Alizarin orange
- Alizarin yellow 3 G
- Alizarin brown
- Anthracene blue

20 When the bath contains .2% ammonia it gives the best results with the above orange and yellow dyes. Alizarin red gives the best result when the bath contains .2% acetic acid. The temperature of the bath may be varied within certain limits, but it is primarily a cold bath in which the gelatin does not soften. The usual working temperatures would be 70° F. After having been dyed the film is washed for about a minute to remove the excess dye, and it has been found that prolonged washing and exposure to light does not affect the dye tones.

It is possible to obtain a pure dye image after the dye is thus mordanted by removing 35 the iron hydroxid with a suitable solvent; and for this purpose I find a 2 per cent. solution of oxalic acid satisfactory. There is left a very transparent dye image. With some dyes it is found that the color of the 40 remaining image is at first somewhat altered, but it is restored to the proper shade by being submitted to running water for a short time.

In place of the bleaching bath first mentioned, the film containing a silver image may 45 be submitted to the following bath:

- Potassium ferricyanid ----- 10,000 grams.
- Ammonia (concentrated .89) ----- 2 liters.
- Water to ----- 200 liters.

50 in which the silver image changes to one of silver ferrocyanid. It is then washed and may be treated with the acid ferrous sulfate bath above mentioned, or with the following bath:

- 55 Ferric ammonium sulfate ----- 2000 grams.
- Potassium bromid ----- 1000 grams.
- Hydrochloric acid (concentrated) ----- 400 cc.
- Water to ----- 200 liters.

60 In either case it is followed by the sodium thiosulfate and sodium carbonate baths above mentioned.

Still a third method of toning is to submit 65 the silver image to the following bath or a

similar one containing ferric ferricyanid in solution:

|                         |             |
|-------------------------|-------------|
| Potassium bichromate    | 5 grams.    |
| Ferric ammonium sulfate | 250 grams.  |
| Oxalic acid             | 600 grams.  |
| Potassium ferricyanid   | 200 grams.  |
| Ammonium alum           | 1000 grams. |
| Hydrochloric acid (10%) | 200 cc.     |
| Water to                | 200 liters. |

70  
75

The image resulting from this bath is presumably one of unchanged silver, silver ferrocyanid and ferric ferrocyanid. The unchanged silver and silver ferrocyanid are removed in a bath of potassium ferricyanid 80 and sodium thiosulfate (the well known Farmer's reducer). The remaining blue image may then be converted into an iron hydroxid image by a bath of sodium carbonate, caustic soda, or the like.

85

While the desired results may be obtained by following the processes as indicated above without a knowledge of the chemistry involved, it may be of interest to note the probable reactions which occur. The reaction between ferrous sulphate and hydrochloric acid in the bath containing them results in the formation of ferrous chlorid. When the silver ferricyanid image, obtained by the first bath, is submitted to the acid 95 ferrous sulfate bath it is presumed that the re-action involved is given by the following reaction:



The silver chlorid thus obtained is removed into hypo and the action of the sodium carbonate bath is presumed to be as follows:



It may be noted, however, that it is very questionable whether the ferrous ferricyanid image obtained is a permanent one, as it is thought highly probable that the oxygen present in the wash water oxidizes it into the ferric condition, so that the image is either one of ferric ferrocyanid or one of the mixed salts.

If the silver ferrocyanid image is first obtained, the acid ferrous sulfate bath in the presence of oxygen converts this to ferric ferrocyanid and silver chlorid.

When, however, the silver image is transformed directly into the complex cyanid of iron image, the re-action involved is supposed to be as follows:



It is understood that in place of sodium carbonate other baths containing hydroxyl ions may be used, in particular solutions of any of the carbonated or caustic alkalis of 130

the alkali elements, lithium, sodium, potassium, and the radical ammonium. Other baths containing ferrous ions may be substituted for the acid ferrous sulfate bath.

- 5 The resulting image of colloidal iron hydroxid is transparent, and the slight color present does not affect the dye image disadvantageously. The process which I have outlined as preferred is advantageous in 10 that a film is not submitted to any bath which tends to abnormally tan or harden the gelatin, by virtue of a combination of the gelatin and iron. The ferrous ions do not appear to have this effect, whereas the ferric ions which are present in those baths which contain a ferric salt have a mordanting effect and there is a tendency for the dye to produce stained highlights in the dyed image. 15
- 20 The resulting colored film was found to be unimpaired in wearing quality, and, by attending to manipulate details given hereinabove, effects can be duplicated with certainty. The image is durable on prolonged exposure, either to water or light. Since the salts resulting in each re-action are formed substantially in correspondence or proportion to the original image and since the dye is adsorbed substantially in proportion to the mordanting salt, the dyed image will have a gradation similar to that of the original image.

While I have outlined above the preferred methods of carrying out this process, it is understood that many changes may be made and the proportions of ingredients may be varied within certain limits, and such changes are contemplated as being within the scope of my invention as defined by the following claims.

Having thus described my invention, what I claim as new and desire to secure by Letters Patent is:

1. The process of producing a colored image from a photographic image, which consists in replacing at least a part of the original photographic image by an iron toned image and mordanting a suitable dye to the toned image.
2. The process of producing a colored image from a silver photographic image, which consists in replacing at least a part of the silver image by an image of an iron salt and in treating said image with a suitable dye until sufficient dye is mordanted thereby to produce a colored image.
3. The process of producing a colored image in gelatin from a silver photographic image, which consists in replacing the silver image by an iron hydroxid image and in mordanting a dye to the iron hydroxid image.
4. The process of producing a transparent colored image in gelatin from a silver photographic image, which consists in trans-

forming the silver image into a colloidal iron hydroxid image and in mordanting thereon an acid dye.

5. The process of producing a transparent colored image in gelatin from a silver photographic image, which consists in replacing at least a part of the silver image by a colloidal iron hydroxid image and in mordanting thereon at normal temperatures an acid dye of the alizarin series. 75

6. The process of producing a colored image in gelatin from a silver photographic image, which consists in transforming the silver image into an image of a complex cyanid of silver and iron, transforming this image into one of a complex cyanid of iron, and then transforming this image into one of iron hydroxid, and mordanting a dye upon the iron hydroxid image. 80

7. The process of producing a mordanted dye image from a silver photographic image that comprises replacing at least a part of the silver image by an image of a complex cyanid of silver and iron, replacing at least a part of this image by one of a complex cyanid of iron, and bathing this in a solution of one of the carbonated or caustic alkalies of the alkali metals including ammonium, and then bathing the resultant image in a suitable dye. 95

8. The method of producing a transparent mordanted dye image from a silver photographic image in a gelatin film that comprises the transforming of the silver image into a silver ferricyanid image, then bathing it first in a solution containing ferrous ions, and then in a solution containing hydroxyl ions and finally in an acid dye of the alizarin series. 100

9. The process of producing a transparent mordanted dye image from a silver photographic image in a gelatin film, which process comprises bathing the film in a solution of potassium ferricyanid and an oxidizing agent, then in an acid solution of ferrous sulfate, then in a solution of sodium thiosulfate and then in a solution containing hydroxyl ions, whereby an image of colloidal iron hydroxid is obtained, and then bathing the film in an acid dye of the alizarin series at a temperature less than 80° F. 105

10. The process of producing in a gelatin film a transparent mordanted dye image from a silver photographic image, which comprises submitting the film containing the silver image to a bath containing potassium ferricyanid and an oxidizing agent, then submitting it to a bath containing ferrous ions, then bathing it in a solution of sodium thiosulfate, and then in a solution containing hydroxyl ions which transforms the image into one of colloidal iron hydroxid, and then mordanting an acid dye to the iron hydroxid image. 110

11. The process of producing a dye image 120

- 4
- from an image composed of an iron salt consisting in mordanting a suitable dye to the image of iron salt and then dissolving the iron salt, leaving the dye image.
- 5 12. The process of producing a transparent dye image in gelatin from a silver photographic image, which consists in replacing the silver image by an iron toned image, mordanting a suitable dye to the iron 10 toned image, and then dissolving out the iron toned image.
13. The process of producing a transparent dye image in gelatin from a silver photographic image, which consists in replacing at least a part of the silver image by an image of colloidal iron hydroxid, treating this image with a suitable acid dye until sufficient dye is mordanted thereby to produce a colored image and then dissolving the iron hydroxid in a solution of oxalic acid, leaving a dye image.
14. The method of transforming a silver photographic image into an iron hydroxid image, which consists of submitting it successively to baths that transform it into a complex cyanid of silver and iron, then into a complex cyanid of iron and then into iron hydroxid.
15. The method of transforming a silver photographic image in gelatin into a transparent colloidal iron hydroxid image capable of mordanting dyes that consists in submitting the silver image to a solution of potassium ferricyanid and an oxidizing agent, then to an acid solution of ferrous sulfate, then to a solution of sodium thiosulfate and finally to a solution containing hydroxyl ions.
16. The method of transforming a silver photographic image into a colloidal iron hydroxid image, which consists in transforming it first into a silver ferricyanid image, then bathing it in a solution containing ferrous ions, and then transforming the resultant image into one of iron hydroxid.
17. A colored photograph comprising a dye image that has been mordanted upon an iron toned image.
18. A colored photographic image consisting of an iron toned and mordant dyed image.
19. A colored photograph comprising a colloid layer containing an iron toned image and combined therewith a selectively mordant dyed image.
20. An article of manufacture comprising a gelatin film containing an image composed of an acid dye mordanted upon iron hydroxid.
21. An article of manufacture comprising a gelatin film containing a transparent photographic image of colloidal iron hydroxid having mordanted thereto an acid dye of the alizarin series.
- Signed at Rochester, New York, this 30th day of April 1919.
- JOHN I. CRABTREE.